

No. 664,060.

Patented Dec. 18, 1900.

J. P. SCHUCH, JR.

PROCESS OF EXTRACTING PRECIOUS METALS FROM THEIR ORES.

(Application filed Dec. 27, 1898.)

(No Model.)



Witnesses

J. Frank Culverwell - By his Attorneys,  
D. T. Halligan, Jr.

John Philip Schuch, Jr., Inventor.

C. A. Snow & Co.

# UNITED STATES PATENT OFFICE.

JOHN PHILIP SCHUCH, JR., OF CRIPPLE CREEK, COLORADO.

## PROCESS OF EXTRACTING PRECIOUS METALS FROM THEIR ORES.

SPECIFICATION forming part of Letters Patent No. 664,060, dated December 18, 1900.

Application filed December 27, 1898. Serial No. 700,405. (No specimens.)

*To all whom it may concern:*

Be it known that I, JOHN PHILIP SCHUCH, Jr., a citizen of the United States, residing at Cripple Creek, in the county of El Paso and 5 State of Colorado, have invented a new and useful Process of Extracting Precious Metals from Their Ores, of which the following is a specification.

This invention relates to an improved process 10 of extracting precious metals from their ores; and it has for one object to provide for treating metal-bearing ores by the use of cyanogen containing solvents in a novel and efficient manner, whereby a much larger percentage 15 of the value of the ores may be saved than has been heretofore possible by the ordinary cyanid process.

Heretofore in treating gold-bearing ores by the common cyanid process the ore is first 20 crushed, dried, and rolled to a proper degree of fineness, and that which requires roasting is then conveyed to the roasters, while the oxidized ore, which does not require roasting, is delivered to the bin or receptacle therefor. 25 After the portion of the ore to be roasted has passed through this step of the process the same is conveyed to the cooling-room before being deposited in the bin or receptacle referred to, which contains the ore requiring no 30 roasting. All of the ore is then removed by manual labor into the ordinary stationary cyanid-tanks, and after these tanks are filled with the ore the cyanid solution is introduced therein. In this process the filled cyanid-tanks, with 35 the solution and ore therein, are permitted to remain filled and unmolested for a sufficient length of time for the solution to act on the ore, after which the gold-bearing solution is drawn off and allowed to flow to the precipitation-room, while the tailings in the tank are 40 then washed with water and shoveled out, or sluiced out when this is possible. In carrying out this old cyanid process the percentage extracted rarely exceeds ninety per cent. 45 of the ore value, whereas the present invention provides a process for saving a larger per cent. of the ore value, while at the same time permitting of the mixing together of various grades of ore with a cyanid solution, so as to 50 make one even grade out of ores of various values.

A further object of the invention is to pro-

vide a process which involves the thorough aeration of the ore and solution during mixing, whereby the oxygen of the air may be utilized 55 to assist in dissolving the gold in the ore.

The process contemplated by the present invention may be carried out by any practical means which would involve the mixing of the cyanid solution with the ore prior to its introduction 60 into the lixiviation-tanks, as this is one of the leading objects of the invention—namely, to overcome the objection to first mixing the ore with the cyanid solution directly in such tanks. However, the preferred 65 manner of carrying out the process is in connection with the improved mixing-machine disclosed in my contemporaneously-pending application, Serial No. 697,780.

The preferred form of mixing machine or 70 apparatus with which the process is carried out is shown in the accompanying drawing, in which the figure is a sectional view thereof.

The mixing-machine illustrated in the drawing essentially consists of an upright tank 1 75 of the required capacity, which is entirely open at the upper end thereof and has connected with the bottom a solution drainage-pipe 9, which leads to the usual precipitation-boxes in the precipitation-room, whereby the 80 gold-bearing solution which percolates to the main bottom of the tank may be conveyed to the precipitation-room to provide for precipitating the precious metal from the solution. The said tank 1 has fitted within the bottom 85 thereof a strainer 10, through which the gold-bearing solution must pass before reaching the drainage-pipe 9, and serves to collect and retain sand, slime, and other impurities contained in the ore or evolved by the chemical 90 action of the cyanid solution thereon. The said strainer 10 therefore effects a separation between the gold-bearing solution and the ore pulp or slush which is mixed with more or less of the solution, as the result of the 95 mixing operation within the mixing-tank, and to provide for carrying off said ore pulp or slush which does not penetrate the strainer the tank 1 has fitted thereto above the plane of the strainer an ore-discharge spout 16, 100 through which the ore pulp or slush, which is necessarily saturated with more or less of the cyanid solution, passes and is delivered into the lixiviation-tanks.

To provide for an intimate mixing of the ore and cyanid solution within the mixing-tank, the latter has arranged therein a revolute agitator 18, and a solution-supply pipe 5 40 is fitted in one side of the tank near the top thereof to provide for delivering into the same a constant stream of the cyanid solution.

Other details of the mixing-machine which are not essential to the present invention are 10 fully described in the other application herein referred to.

Now in the ordinary process of treating gold-bearing ores, as explained in the statement of invention, the oxidized ore which has 15 been crushed and reduced to a proper degree of fineness does not need roasting, while other portions of the ore must be subjected to the roasting step. In the present invention, however, instead of allowing the roasted ore to 20 become entirely cold in the cooling-room the same is conveyed or delivered by a conveyer or any suitable means through a feed-chute 38 directly into the open upper end of the mixing-tank 1 while the ore is still in a warm 25 condition. At the same time a stream of the oxidized ore is delivered from this receptacle by any suitable means, preferably through a feed-chute 39, into the open upper end of the mixing-tank. While the separate portions of 30 the ore are thus being delivered into the mixing-tank a constant stream of the cyanid solution is also being delivered into the tank by the solution-supply pipe 40, previously referred to, and as the agitator 18 is constantly 35 revolved in the tank the entire mass of ore is intimately mixed with the solution, thereby insuring an even and uniform extraction of the precious metals from their ores. As previously explained, the gold-bearing cyanid 40 solution passes through the strainer in the bottom of the tank and into the solution-drainage pipe 9, through which it is carried to the precipitation - room, while the ore slush or pulp, mixed with the solution, discharges 45 through the spout 16 and is delivered to the lixiviation-tanks. So it will be observed that the ore is thoroughly mixed with the cyanid solution prior to its introduction into the lixiviation-tanks.

50 In carrying out the invention it is necessary that the ore and cyanid solution while being mixed together must be thoroughly aerated or charged with air, so that the oxygen from the air will assist in dissolving the gold in the ore. By using the cyanid solution instead of water on the ore at the stamp-mills it is unnecessary to charge the mixture within the mixing-tank with air. In fact, the free-gold ores or oxidized ores can be treated 55 through the stamp-mill by using the cyanid solution instead of water, and the solution, carrying the fine ore with it, may be either run over amalgamating-plates directly to the cyanid-tanks or to the mixing-tank, herein described; but in either event it will be seen that by mixing the cyanid solution with the ore directly at the stamp-mill the mixture

will be necessarily exposed to the air, so that the oxygen in the air will be free to assist in dissolving the gold in solution. However, in 70 the preferred way of carrying out the invention it is necessary to charge the mixture within the mixing-tank with air, and to accomplish this the tank is provided, preferably near the top thereof, with an exterior 75 annular air-blast pipe 41, having a plurality of dependent jet-pipes 42, opening into the tank near the bottom thereof, so as to inject air into the mixture of ore and solution during the mixing thereof by the agitator. 80

In connection with the aeration of the ore and cyanid solution the best results are accomplished by using hot air. The use of hot air is specially practical in connection with the jet-pipes of the mixing-tank, and heated 85 air should always be forced into the ore within the mixing-tank when the ore is cold or not roasted.

Another feature of importance in carrying out the process is to use the cyanid solution 90 quite warm, and a number of expedients may be resorted to for the purpose of maintaining the solution at a proper temperature. As the ore which is introduced into the tank 1 of the mixing-machine is used while in a warm condition, the same will necessarily serve to keep the cyanid solution warm, so that ordinarily in connection with the mixing-machine it will not require supplemental means for heating up the cyanid solution; but as it may be necessary at times to resort to supplemental means for heating the solution before introducing it into the mixing-tank one way to accomplish this result is illustrated in the drawing, where the solution - supply pipe 40 is 95 shown leading from a storage tank or reservoir 46 for the cyanid solution. This storage tank or reservoir 46 may have arranged therein a heating-coil 47 of piping, the terminals of which coil are connected with any suitable 100 supply for steam or hot air, whereby a circulation of steam or hot air may be maintained in the coil, thus insuring the thorough heating up of the cyanid solution before it is delivered through the supply pipe or pipes to 105 the point of use. While the interior heating-coil within the storage tank or reservoir for the cyanid solution will accomplish the desired result, it will be understood that an exterior coil or any extraneous means for heating 110 up the solution may be utilized for the same purpose.

In the practical operation of the process it has been found that the best results are accomplished by heating the air when the same 125 is introduced through the jet-pipes 42 into the mixture, inasmuch as air in a heated condition has been proven to be very effective to insure the active attacking and dissolving of the gold by the cyanid solution.

130 It has already been explained that ordinarily a separate heating of the solution which is used in the mixing-tank is not necessary; but this is always necessary when the cyanid

solution is used at the stamp-mill or in any wet crushing-machine instead of water, which operation dispenses with the necessity of introducing air into the mixture within the mixing-tank, as previously explained.

It will of course be understood that when the cyanid solution is used in a warm condition directly at the stamp-mill or in any wet crushing-machine said cyanid solution may 10 be heated up in the storage tank or reservoir in the same manner illustrated in the figure of the drawing, the essential feature of this particular process residing in having the solution in a thoroughly-heated condition, yet 15 below the point of boiling or evaporation.

While the essential features of the process have already been indicated, it will be understood that in carrying out the same quicksilver can be used at any point where free 20 gold is present—such, for instance, as on plates in the stamp-mill or on any wet crushing-machine, or also on specially-constructed pans or prepared plates within the mixing-machine herein referred to—so as to insure 25 the collecting of all coarse free gold.

In carrying out the herein-described process in the precipitation of the gold from the cyanid solution any method may be used, such as the zinc-shavings method, electrolysis, or the charcoal method, &c.

30

Having thus described the invention, what is claimed as new, and desired to be secured by Letters Patent, is—

A method of extracting precious metals from their ores, which consists in combining the crushed ore with a cyanid solution while both are in a warm condition, mechanically mixing the ore and solution by agitation simultaneously with the commingling thereof, charging the mixture during the agitation 35 with hot air, and finally separating the ore and slush or pulp from the metal in solution, substantially as set forth.

In testimony that I claim the foregoing as my own I have hereto affixed my signature in 40 the presence of two witnesses.

JOHN PHILIP SCHUCH, JR.

Witnesses:

F. H. NOLTE,

A. B. OLSON.